

# United States Patent

## Schevey

[15] 3,661,731

[45] May 9, 1972

### [54] ELECTRODEPOSITION OF BRIGHT NICKEL

[72] Inventor: William R. Schevey, Hawley, Pa.  
[73] Assignee: Allied Chemical Corporation, New York, N.Y.  
[22] Filed: Mar. 16, 1970  
[21] Appl. No.: 20,031

[52] U.S. Cl.....204/49  
[51] Int. Cl. ....C23b 5/08  
[58] Field of Search.....204/49, 43, 44

### [56] References Cited

#### UNITED STATES PATENTS

3,219,559 11/1965 Ostrow et al.....204/49  
3,305,461 2/1967 Ostrow et al.....204/49

3,305,462 2/1967 Ostrow et al.....204/49  
3,306,831 2/1967 Cope, Jr. ....204/43  
3,312,604 4/1967 Wells et al. ....204/49  
3,429,789 2/1969 Ostrow et al.....204/49

Primary Examiner—G. L. Kaplan  
Attorney—Ernest A. Polin

[57]

### ABSTRACT

Acid nickel plating bath for obtaining bright nickel deposits, said bath being of the chloride, sulfate, fluoborate or sulfamate type and containing a brightener mixture comprising the disodium salt of methylene bis naphthalene sulfonic acid and a second component selected from coumarin, piperonal bisulfite complex, sodium beta-styrene sulfonate, benzimidazole and mixtures thereof, with the proviso that benzimidazole is used only when greater than 50 mole percent of nickel salt used in the bath is nickel fluoborate.

13 Claims, No Drawings

## ELECTRODEPOSITION OF BRIGHT NICKEL

## BACKGROUND OF THE INVENTION

Acid nickel plating baths normally yield dull electrodeposits, but bright deposits can be obtained by the addition of effective amounts of certain organic compounds, known as brighteners.

It is the object of this invention to provide a novel mixture of brighteners for use in acid nickel plating baths.

It is a further object to provide improved acid nickel bath compositions for bright nickel plating.

It is still another object to provide an improved method for obtaining bright nickel electrodeposits.

## SUMMARY OF THE INVENTION

It has been discovered that when both Brightener A and Brightener B, defined below, are added in sufficient amounts to a conventional acid nickel plating bath of the sulfate, chloride, fluoborate or sulfamate type, a bright nickel electrodeposit is obtained which is superior to the deposit obtained when only one of Brightener A or Brightener B is added to the bath.

The plating bath comprises an aqueous acid solution of 25 nickel salt selected from the group consisting of nickel sulfate, nickel chloride, nickel fluoborate, nickel sulfamate or mixtures thereof.

Brightener A is the disodium salt of methylene bis naphthalene sulfonic acid and has the structural formula:



wherein each  $\text{SO}_3\text{Na}$  group can replace any one hydrogen atom in each naphthalene group.

Brightener B is selected from the group consisting of:

1. coumarin, having the structural formula:



2. piperonal bisulfite complex, having the structural formula:



3. sodium beta-styrene sulfonate, having the structural formula:



4. benzimidazole, having the structural formula:



5. mixtures thereof, with the proviso that benzimidazole is used only when greater than 50 mole percent of nickel salt used in the bath is nickel fluoborate. Preferably benzimidazole is used only when greater than about 80 mole percent of nickel salt is nickel fluoborate.

## DETAILED DESCRIPTION

Brightener A and Brightener B are each added to the plating bath in amounts sufficient to obtain a bright nickel electrodeposit. Generally, the concentrations of Brightener A and of Brightener B dissolved in the nickel plating bath independently range from about 0.1 to about 10 grams per liter of plating bath, but not exceeding the saturation concentration thereof. Although some of the brightener compounds have 10 saturation concentrations greater than 10 grams per liter, no advantage is seen from the use of such higher concentration. Preferably the concentrations of Brightener A and Brightener B independently range from about 0.12 to about 2.0 grams per liter but not exceeding the saturation concentration thereof.

15 While Brightener A and Brightener B can each be added to the nickel plating bath separately, it is preferred that they first be premixed, so that they can be added to the bath in one step. This mixture, called the "brightener mixture", should contain sufficient amounts of Brightener A and Brightener B so that when the mixture is added to the plating bath, the above indicated bath concentrations will be satisfied.

A convenient method of adding the brightener mixture to the plating bath is to first prepare a solution of the brightener mixture, and then add said solution to the plating bath. The solvent used in preparing the solution of brightener mixture should be soluble in the plating bath. Preferably the solvent is selected from the group consisting of water, aliphatic monohydric alcohols having from one to three carbon atoms 30 and mixtures thereof. The aliphatic monohydric alcohols are methanol, ethanol, n-propanol and isopropanol, with isopropanol being preferred. When the brightener mixture includes coumarin, it is preferred that the solvent contain at least 25 volume percent alcohol.

35 The ratio of Brightener A to Brightener B in the brightener mixture or dissolved in the bath is not critical, but generally the weight ratio varies from about 0.1:1 to about 10:1, preferably from about 0.5:1 to about 2:1.

40 The brightener mixtures of this invention are generally compatible with addition agents conventionally employed in plating baths, for example, wetting agents, such as sodium lauryl sulfate and castile soap, antifoam agents, stress relief agents and the like.

45 It is a preferred embodiment of this invention that the brightener mixtures be used in conjunction with saccharin. Saccharin has the effect of reducing the stress and brittleness of the nickel deposit and also somewhat increases the brightness of the deposit. Generally, the concentration of 50 saccharin ranges from about 0.1 gram per liter of plating bath to its saturation concentration, preferably from about 0.5 to about 2.0 grams per liter of plating bath.

55 Saccharin may be added to the bath separately or it may first be incorporated as part of the brightener mixture. In the latter case, the amount of saccharin in the brightener mixture is not critical as long as the amount is sufficient to supply the above indicated concentrations of saccharin in the bath. Generally, the weight ratio of saccharin to brightener mixture varies from about 0.1:1 to about 10:1, preferably from about 1:1 to about 8:1.

60 The bright nickel deposit is obtained in conventional manner by passing a current through a nickel plating bath containing Brightener A and Brightener B, between the anode, which is typically nickel, and the cathode, which is the article to be plated.

65 Temperature, current density, pH, and other operating conditions are relevant only as far as they influence the basic characteristics of the plating bath in known manner. Thus 70 operating conditions commonly employed with the conventional nickel plating solutions may be employed when those solutions contain the brightener mixtures.

Generally, plating bath temperatures may vary from about 40° to about 170° F., preferably from about 90° to about 140° F.

Current density generally ranges from about 1 to about 300 amps per square foot, preferably from about 10 to about 150 amps per square foot. For plating of wires, current densities as high as 600 amps per square foot can be employed. With Watts Nickel type baths, however, lower current densities are generally employed, usually up to about 80 amps per square foot, with up to about 100 amps per square foot for wires.

Values for bath pH generally range from about 2.5 to about 5.0, preferably from about 3.5 to about 4.5. A bath pH between about 5.0 and about 7.0 can also be employed, but at these pH values, the bath usually requires the addition of nickel complexing agents, e.g. citric acid, malic acid or ammonium hydroxide.

It is preferred that during the plating process relative movement be provided between the plating bath and the object being plated. Any conventional means for agitating the bath or for moving the object being plated may be employed. Illustrative of such means are mechanical stirring of the bath, passage of compressed air through the bath, cathode rod agitation, and the like.

The baths listed in the following table illustrate, but do not limit, the types of electroplating baths in which the brightener mixtures of this invention may be incorporated as addition agents in the above indicated proportions. The composition ranges generally employed in the art are stated for each of the baths in grams per liter of bath.

TABLE I

|                                                   |                     |  |
|---------------------------------------------------|---------------------|--|
| 1. Nickel Fluoborate Bath                         |                     |  |
| Ni(BF <sub>4</sub> ) <sub>2</sub>                 | 4-680 grams/liter   |  |
| Boric Acid                                        | 30-50 grams/liter   |  |
| 2. Watts Nickel Type Bath                         |                     |  |
| NiSO <sub>4</sub> ·6H <sub>2</sub> O              | 135-400 grams/liter |  |
| NiCl <sub>2</sub> ·6H <sub>2</sub> O              | 30-75 grams/liter   |  |
| Boric Acid                                        | 30-50 grams/liter   |  |
| 3. Nickel Sulfamate Bath                          |                     |  |
| Ni(NH <sub>2</sub> SO <sub>3</sub> ) <sub>2</sub> | 300-450 grams/liter |  |
| Boric Acid                                        | 30-50 grams/liter   |  |
| 4. Nickel Chloride Bath                           |                     |  |
| NiCl <sub>2</sub> ·6H <sub>2</sub> O              | 150-300 grams/liter |  |
| Boric Acid                                        | 30-50 grams/liter   |  |
| 5. Nickel Sulfate Bath                            |                     |  |
| NiSO <sub>4</sub> ·6H <sub>2</sub> O              | 75-200 grams/liter  |  |
| Boric Acid                                        | 30-50 grams/liter   |  |

The above nickel baths generally may contain minor amounts of other nickel salts. For example, the above fluoborate bath may additionally contain nickel chloride or nickel sulfate, usually in such amounts that at least about 80 mole percent of the nickel salt is nickel fluoborate.

The preferred bath is a nickel fluoborate bath wherein the nickel fluoborate concentration ranges from about 220 to 440 grams per liter, especially wherein at least about 80 mole percent of the nickel salt is nickel fluoborate.

The invention can be more fully understood by reference to the following examples.

## EXAMPLE 1

Tests were carried out in a heated 267 ml Hull Cell, plating onto brass Hull Cell panels. All samples were compared at one to two amps. The plating solution was a nickel fluoborate solution having the following characteristics:

|                                   |                 |
|-----------------------------------|-----------------|
| Ni(BF <sub>4</sub> ) <sub>2</sub> | 440 grams/liter |
| pH                                | 4               |
| Temperature                       | 110° F.         |

Runs were made both with and without air agitation of the 70 solutions.

The various brighteners used and descriptions of the resultant plates are listed in Table II below. In Table II the units "g/l" refer to grams of brightener per liter of plating bath. The term "Tanol N" is a trademark for a mixture of dis-

odium salts of methylene bis naphthalene sulfonic acid. The term "Heloplex" is a trademark for piperonal bisulfite complex.

TABLE II

|    | Brightener                                   | Plate Description                      |
|----|----------------------------------------------|----------------------------------------|
| 10 | 1) Blank                                     | Dull                                   |
|    | 1A) Blank plus agitation                     | Dull                                   |
|    | 2) .15 g./l. Tamol N                         | Bright below 20 amps/sq. ft.           |
|    | 2A) .15 g./l. Tamol N                        | Bright below 20 amps/sq. ft.           |
|    | Plus agitation                               |                                        |
| 15 | 3) .15 g./l. Tamol N                         | Semi-bright                            |
|    | 1.0 g./l. saccharin                          |                                        |
|    | 3A) .15 g./l. Tamol N                        | Semi-bright                            |
|    | 1.0 g./l. saccharin                          |                                        |
|    | Plus agitation                               |                                        |
| 20 | 4) .15 g./l. coumarin                        | Dull                                   |
|    | 4A) .15 g./l. coumarin                       | Dull with bright spots                 |
|    | Plus agitation                               |                                        |
| 25 | 5) .15 g./l. coumarin                        | Bright with gas bubble streaks         |
|    | .15 g./l. Tamol N                            | Bright                                 |
|    | .15 g./l. Tamol N                            |                                        |
|    | Plus agitation                               |                                        |
| 30 | 6) .15 g./l. coumarin                        | Bright, but pitted                     |
|    | .15 g./l. Tamol N                            |                                        |
|    | .15 g./l. saccharin                          |                                        |
|    | 6A) .15 g./l. coumarin                       | Bright                                 |
|    | .15 g./l. Tamol N                            |                                        |
|    | .15 g./l. saccharin                          |                                        |
|    | Plus agitation                               |                                        |
| 35 | 7) .15 g./l. benzimidazole                   | Dull with bright spots                 |
|    | 7A) .15 g./l. benzimidazole                  | Dull with bright spots                 |
|    | Plus agitation                               |                                        |
| 40 | 8) .15 g./l. Tamol N                         | Bright                                 |
|    | .15 g./l. benzimidazole                      |                                        |
|    | 8A) .15 g./l. Tamol N                        | Bright                                 |
|    | .15 g./l. benzimidazole                      |                                        |
|    | Plus agitation                               |                                        |
| 45 | 9) .15 g./l. Tamol N                         | Bright, put pitted                     |
|    | .15 g./l. benzimidazole                      |                                        |
|    | 9A) .15 g./l. Tamol N                        | Bright                                 |
|    | .15 g./l. saccharin                          |                                        |
|    | Plus agitation                               |                                        |
| 50 | 10) .15 g./l. sodium beta-styrene sulfonate  | Semi-bright                            |
|    | 10A) .15 g./l. sodium beta-styrene sulfonate | Semi-bright                            |
|    | Plus agitation                               |                                        |
| 55 | 11) .15 g./l. Tamol N                        | Semi-bright (but brighter than run 10) |
|    | .15 g./l. sodium beta-styrene sulfonate      |                                        |
|    | 11A) .15 g./l. Tamol N                       | Bright                                 |
|    | .15 g./l. sodium beta-styrene sulfonate      |                                        |
|    | Plus agitation                               |                                        |
| 60 | 12) .15 g./l. Tamol N                        | Bright                                 |
|    | .15 g./l. sodium beta-styrene sulfonate      |                                        |
|    | 1.0 g./l. saccharin                          |                                        |
|    | 12A) .15 g./l. Tamol N                       | Bright                                 |
|    | .15 g./l. sodium beta-styrene sulfonate      |                                        |
|    | 1.0 g./l. saccharin                          |                                        |
|    | Plus agitation                               |                                        |
| 65 | 13) .15 g./l. Heloplex                       | Dull, bright streak at 12 amps/sq. ft. |
|    | 13A) .15 g./l. Heloplex                      | Dull with bright streak                |
|    | Plus agitation                               |                                        |
| 70 | 14) .15 g./l. Tamol N                        | Bright, but pitted                     |
|    | .15 g./l. Heloplex                           |                                        |
|    | 14A) .15 g./l. Tamol N                       | Bright                                 |
|    | .15 g./l. Heloplex                           |                                        |
|    | Plus agitation                               |                                        |
| 75 | 15) .15 g./l. Tamol N                        | Bright                                 |
|    | .15 g./l. Heloplex                           |                                        |
|    | 1.0 g./l. saccharin                          |                                        |
|    | 15A) .15 g./l. Tamol N                       | Bright                                 |
|    | .15 g./l. Heloplex                           |                                        |
|    | 1.0 g./l. saccharin                          |                                        |
|    | Plus agitation                               |                                        |
|    | 16) .15 g./l. coumarin                       | Dull                                   |
|    | .15 g./l. sodium beta-styrene sulfonate      |                                        |
|    | 16A) .15 g./l. coumarin                      | Dull with bright spots                 |
|    | .15 g./l. sodium beta-styrene sulfonate      |                                        |

|      |                         |                        |
|------|-------------------------|------------------------|
| 17)  | Plus agitation          | Dull with bright spots |
|      | .15 g./l. Heloplex      |                        |
|      | .15 g./l. coumarin      |                        |
| 18)  | .15 g./l. Heloplex      | Dull with bright spots |
|      | .15 g./l. coumarin      |                        |
|      | 1.0 g./l. saccharin     |                        |
| 19)  | .15 g./l. Heloplex      | Bright streaks         |
|      | .15 g./l. benzimidazole |                        |
| 20)  | .15 g./l. Heloplex      | Dull with bright spots |
|      | .15 g./l. benzimidazole |                        |
|      | 1.0 g./l. saccharin     |                        |
| 20A) | .15 g./l. Heloplex      | Dull with bright spots |
|      | .15 g./l. benzimidazole |                        |
|      | 1.0 g./l. saccharin     |                        |
|      | Plus agitation          |                        |

## EXAMPLE 2

The tests of Example 1 are repeated using a Watts Nickel type bath having the following characteristics:

|                                     |                 |
|-------------------------------------|-----------------|
| NiSO <sub>4</sub> 6H <sub>2</sub> O | 300 grams/liter |
| NiCl <sub>2</sub> 6H <sub>2</sub> O | 45 grams/liter  |
| Boric Acid                          | 30 grams/liter  |
| pH                                  | 4               |
| Temperature                         | 110° F.         |

Results substantially similar to those of example 1 are obtained, except that no brightening is observed when brightener mixtures containing benzimidazole are used.

## EXAMPLE 3

The tests of example 1 are repeated using a nickel sulfamate bath having the following characteristics:

|                                                   |                 |
|---------------------------------------------------|-----------------|
| Ni(NH <sub>2</sub> SO <sub>3</sub> ) <sub>2</sub> | 300 grams/liter |
| Boric Acid                                        | 30 grams/liter  |
| pH                                                | 4               |
| Temperature                                       | 110° F.         |

Results substantially similar to those of example 1 are obtained, except that no brightening is observed when brightener mixtures containing benzimidazole are used.

I claim:

1. In a bath for the electrodeposition of nickel, comprising an aqueous acid solution of nickel salt selected from the group consisting of nickel fluoborate, nickel chloride, nickel sulfate,

nickel sulfamate and mixtures thereof, the improvement which comprises incorporating therein, in amounts sufficient to obtain a bright nickel deposit, the disodium salt of methylene bis naphthalene sulfonic acid (Brightener A) and a 5 component selected from the group consisting of coumarin, piperonal bisulfite complex, sodium beta-styrene sulfonate, benzimidazole and mixtures thereof (Brightener B), with the proviso that benzimidazole is used only when greater than 50 mole percent of nickel salt used in the bath is nickel 10 fluoborate.

2. The bath of claim 1 wherein the concentrations of Brightener A and Brightener B independently range from about 0.1 to 10 grams per liter of bath, but not exceeding their saturation concentrations.

15 3. The bath of claim 2 wherein greater than 50 mole percent of nickel salt used in the bath is nickel fluoborate and Brightener B is benzimidazole.

4. The bath of claim 3 wherein greater than 80 mole percent of the nickel salt is nickel fluoborate.

20 5. The bath of claim 2 wherein Brightener B is coumarin.

6. The bath of claim 2 wherein Brightener B is piperonal bisulfite complex.

7. The bath of claim 2 wherein Brightener B is sodium beta-styrene sulfonate.

25 8. The bath of claim 2 which additionally contains saccharin in a concentration ranging from about 0.1 gram per liter to its saturation concentration.

9. The bath of claim 1 wherein the concentrations of Brightener A and Brightener B independently range from

30 about 0.12 to 2.0 grams per liter of bath, but not exceeding their saturation concentrations.

10. The bath of claim 9 wherein at least about 80 mole percent of the nickel salt is nickel fluoborate and the nickel fluoborate concentration ranges from about 220 to about 440

35 grams per liter of bath.

11. The bath of claim 9 which additionally contains saccharin in a concentration ranging from about 0.5 to about 2.0 grams per liter of bath.

40 12. A nickel plating process comprising passing a current from an anode to a cathode through the bath of claim 1.

13. A nickel plating process comprising passing a current from an anode to a cathode through the bath of claim 8.

\* \* \* \* \*

45

50

55

60

65

70

75